

# UNITED STATES PATENT OFFICE.

ARCHIBALD CLAUDE EVANS, OF HAMPTON WICK, AND PERCY JOSÉ MITCHELL, OF  
WESTMINSTER, LONDON, ENGLAND.

## BINDING COMPOUND AND PROCESS OF MAKING SAME.

1,209,692.

Specification of Letters Patent. Patented Dec. 26, 1916.

No Drawing.

Application filed September 7, 1915. Serial No. 49,349.

*To all whom it may concern:*

Be it known that we, ARCHIBALD CLAUDE EVANS and PERCY JOSÉ MITCHELL, residing at Hampton Wick, Middlesex, England, and Westminster, London, England, respectively, have invented certain new and useful Improvements in Binding Compounds and Processes of Making Same; and we do hereby declare the following to be a full, clear, and exact description of the invention, such as will enable others skilled in the art to which it appertains to make and use the same.

This invention relates to a new and improved binding material for use in briquetting, road making and the like applications and comprises a process for producing same.

Heretofore tar pitch has been the binding agent or ingredient mostly employed for the purpose of making fuel briquets from coal, and while its use is very effective for such purpose the same is attended by a number of disadvantages. Among these may be mentioned firstly the fact that operatives employed in the process using pitch are subject to pitch cancer, and skin troubles due probably to the presence of phenols or phenol derivatives which escape from the molten compound. A further disadvantage is that in order to obtain the pitch the tar has to be subjected to a prolonged and therefore costly process of distillation before it will yield a substance that will set to a sufficient hardness when cold. The necessity of carrying out this distillation accounts for the presence of the phenols in the finished product, the reason being that although these phenols are removed in the earlier stages of distillation it is necessary to introduce a portion of the first runnings into the still at the close of the distillation in order to be able to withdraw the thick pitch which remains, and it is in this way that the phenols are introduced into the product.

Processes have already been proposed for solidifying tar by heating it in a still to a temperature not exceeding 360° F. and after cooling adding to it considerable quantities of sulfuric acid, these quantities varying from a minimum of 3% to a maximum of 12½%. The present invention differs from such previously known processes in that in the latter practically the whole of the solidifying is effected by means of a considerable

quantity of sulfuric acid, while in the former the solidification is effected principally by the addition of a considerable quantity of carbon, while only an exceedingly small quantity of sulfuric acid is used at the end of the process; it will thus be apparent that the material obtained according to the present invention will be of an entirely different character to that above referred to.

Now according to this invention a binding material for use in briquetting, road making and the like is produced from coal tar or mineral oil products without the necessity for the prolonged and complete distillation above referred to. Further a greatly increased yield of binding material from a given quantity of tar is obtained as compared with the amount of pitch which the tar would yield in the ordinary way. The phenols removed in the earlier distillation are not re-introduced into the product and the process also provides means for regulating the ultimate consistency and binding properties of the finished product.

The invention is carried out as follows: The starting out material is preferably coal tar in the condition in which the same is usually obtained from gas works except that most of the ammonia may have been removed from the tar before use. The tar is distilled at a temperature of 270° in a suitable retort or still. The latter may be of any convenient type but should be fitted with a man-hole capable of being hermetically closed and should further be provided with a mechanical stirring device. The heating arrangements consist preferably of a furnace provided with the usual flues which should be so arranged that the heat can be shut off at any desired moment, so as to allow the contents of the still to cool. The distillation is carried on until the light oils have been removed but not to such a point that the anthracene grease passes over. The heat is now shut off and the contents of the still allowed to cool to a temperature below 250° C. This temperature should be as near 250° C. without actually reaching it as possible. Coal dust or hydrocarbon soot *i. e.* soot containing volatile matter, in an impalpable form is now gradually added and stirred into the mass. The reason why this operation must not be carried out at a temperature above 250° C. is, that as the man-

hole must be opened for the purpose the tar and coal dust would be liable to catch fire if this temperature were exceeded. The coal used should preferably be of high volatile 5 contents and the amount added may be varied according to the density and hardness of the finished product required. For the briquetting material from 2½% to 15% of coal or hydro-carbon soot is a working material. For road making the percentage may be increased up to 30%. As soon as the whole of the coal or soot has been added the man-hole is again closed and the temperature raised to a minimum of 270° stirring 10 being continued the whole time; the content is kept at that temperature or not lower than that temperature until the added coal or like material begins to soften and give off its volatile contents. As soon as this action 15 starts the heat is immediately shut off and the material is allowed to cool as rapidly as possible to a temperature below 100° C. If desired the material can be pumped into a tank or like vessel for this cooling to take 20 place. At this stage 0.25% to 1% of sulfuric acid of a preferred strength of 170° Twaddle is gradually added and intimately mixed with the material and if this operation is carried out in a second tank the latter 25 should be provided with suitable stirring or agitating means. Care must be taken that the temperature of the mixture while the sulfuric acid is being added does not rise above 100° C. nor fall below 49° C. After the 30 acid to its measure has been added and thoroughly stirred in the hot mass is run off and allowed to cool and solidify in any suitable molds or other receptacles convenient for the purpose.

35 40 In lieu of coal tar, shale oil, or any other similar mineral oil may be used, and in the treatment of the same for the purpose of this invention the light volatile oils are distilled off until the residue is of about the same consistency as that of the tar previously referred to at a temperature of 270° C. after the same has been distilled at that temperature in the manner described. The subsequent manufacture of the compound is 45 identical with that described in the case of coal tar. Also in place of sulfuric acid, chlorid of sulfur or other known thickening agent may be employed, but sulfuric acid will generally be found to be preferable, owing 50 to the ease with which it can be procured and owing to the fact that it is less unpleasant to handle than the other known and hitherto used thickening agents.

55 By the above described means a material 60 is produced which resembles pitch and has similar softening and melting points, while its vaporization point is about 70° C. higher than that of most of the ordinary commercial medium pitches usually sold for briquetting purposes. The yield of ordinary pitch

from ordinary coal tar is about 5 tons from 10 tons of tar, while according to the invention 8 tons and 16 cwt. of binding agent can be produced from 10 tons of tar.

Apart from the other previously described 70 advantages of this invention it will be seen that a material which solidifies into a pitch like substance which melts and softens at similar temperatures to pitch is obtained without the necessity of carrying the distillation of the tar to anything like the same stage. A further advantage is that the consistency of the final product can be controlled within reasonable limits by the amount of loading material added. It will 75 also be seen that the objectionable addition of the light oils containing phenols which is usual in the ordinary production of pitch is obviated according to this invention and that the finished product is free from or 80 practically free from phenols which pass over during the first distillation.

We claim:—

1. A process for the manufacture of binding materials for briquetting, road making 90 and the like which includes removing the light oils from coal tar, treating said tar while hot with finely divided coal dust or hydrocarbon soot, cooling the resulting product to 100° C. and then treating with a 95 small quantity of thickening agent.

2. A process for manufacturing binding materials for briquetting, road making and the like which includes distilling coal tar at a temperature of 270° C. until the light 100 oils have been removed, cooling the product to approximately 250° C., adding finely divided coal dust or hydrocarbon soot, stirring the mixture and heating to a minimum temperature of 270° C. until the volatile matter 105 begins to pass off from the added material, cooling the mixture to 100° C. and adding a small quantity of sulfuric acid or a specified equivalent thickening agent.

3. A process for the manufacture of binding materials for briquetting, road making and the like which includes removing the light oils from shale oil distillate or its specified equivalent, treating the same while hot with finely divided coal dust or its specified equivalent, cooling the mixture to 100° C., and adding a small quantity of sulfuric acid or its specified equivalent thickening agent.

4. A process for the manufacture of binding materials for briquetting, road making and the like which includes distilling shale oil distillate or its specified equivalent at a temperature of 270° C. until the light oils 120 have been removed, cooling the product to 125 approximately 250° C., adding finely divided coal dust or its specified equivalent, thoroughly stirring the mixture and heating the same to a minimum temperature of 270° C., maintaining the temperature of 270° C. 130

until the volatile matter of said added material begins to pass off, cooling the mixture to 100° C., and adding a small quantity of sulfuric acid or its specified equivalent thickening agent.

5. A binding material for briquetting, road making and the like consisting of the residue from coal tar after the light oils have been removed, said residue being thickened 10 with coal dust or its specified equivalent and

a small quantity of sulfuric acid or its specified equivalent.

In testimony whereof we affix our signatures in presence of two witnesses.

ARCHIBALD CLAUDE EVANS.  
PERCY JOSÉ MITCHELL.

Witnesses:

FRANK B. DEHN.  
ALBERT R. RAMSEY.